

# UNITED STATES PATENT OFFICE.

ARMIN EICHLER, OF NEW YORK, N. Y.

## PAPER AND FABRIC.

1,218,599.

No Drawing.

Specification of Letters Patent.

Patented Mar. 6, 1917.

Application filed June 28, 1916. Serial No. 106,346.

*To all whom it may concern:*

Be it known that I, ARMIN EICHLER, a citizen of the United States, residing at New York, in the county of New York and State of New York, have invented certain new and useful Improvements in Papers and Fabrics, of which the following is a specification.

This invention relates to the manufacture 10 of sheet materials which have waterproof qualities and in some instances are in imitation of leather.

It is one of the objects of the invention to provide a paper sheet or fabric that will 15 not only be waterproof but which will not crack or become permanently wrinkled in ordinary use and will also be comparatively inexpensive to manufacture.

Another object of the invention is to provide 20 a coated fabric in imitation of leather which will possess many of the desirable characteristics of a rubberized fabric.

Another object of the invention is to provide 25 an inexpensive transparent paper of unusual strength and durability which will not lose its tensile strength or transparency where wrinkled or folded.

Other objects and the features of novelty 30 will become apparent from the following description.

I have discovered that by impregnating a sheet of paper or other absorbent fabric of a flexible nature, such as a woven fabric, with a solution or mixture containing polymerized cumarone and a vegetable oil, the sheet will be rendered waterproof, and in the case of a woven fabric will have the property of straightening out into a flat sheet after having been crumpled, in much 40 the same manner as a sheet of rubber will straighten out. This property gives to the fabric greater durability because it will withstand bending and creasing without breaking the fibers. In the case of a sheet 45 of paper the tensile strength is increased as much as eighty per cent. and the sheet rendered transparent. Folding the sheet does not affect its tensile strength or transparency.

The sheets are also rendered highly acid- 50 and alkali-resisting, in hot or cold solutions; they are unaffected by boiling water, or the like.

As an illustration of one method of practising the invention I heat a quantity of a 55 vegetable oil, such as China wood oil, linseed

oil, poppy seed oil or soy bean oil and add the polymerization products of the cumarone and indene group until the mixture is of the desired consistency. Ordinarily the proportion of cumarone and indene is at least one half the amount of oil and this results in a hard homogeneous mass when cold. This is heated and mixed with a volatile solvent such as one of the commonly used hydrocarbon solvents to form a liquid. The consistency of this liquid mixture will vary in accordance with the material to which it is to be applied. For paper a very thin mixture is used and the paper may be dipped 60 into the mixture or the latter may be applied with a brush or in any other suitable manner. The volatile solvent evaporates and leaves the paper impregnated with the mixture of oil and cumarone.

Woven fabrics may be treated in the manner above described. When an imitation of leather is desired the fabric is impregnated and also coated with a similar mixture to which the requisite pigment has been added. 70

Having thus described my invention, what I claim and desire to secure by Letters Patent is:

1. A new article of manufacture consisting of a sheet of absorbent material impregnated 85 with a mixture containing a vegetable oil and polymerized cumarone.

2. A new article of manufacture consisting of a sheet of absorbent material impregnated with a mixture containing a vegetable oil 90 and the polymerization products of the cumarone and indene groups.

3. A new article of manufacture consisting of a flexible sheet of absorbent material, having applied thereto a mixture containing 95 China wood oil and the polymerization products of the cumarone and indene groups.

4. A new article of manufacture consisting of a flexible sheet of absorbent material, having applied thereto a mixture containing 100 a vegetable oil and the polymerization products of the cumarone and indene groups.

5. A new article of manufacture consisting of a fabric, having applied thereto a mixture containing China wood oil and the 105 polymerization products of the cumarone and indene groups.

6. A new article of manufacture consisting of a fabric, having applied thereto a mixture containing a vegetable oil and the 110 polymerization products of the cumarone and indene groups.

7. A new article of manufacture consisting of a sheet of paper impregnated with a mixture containing China wood oil and the polymerization products of the cumarone and indene groups. 5
8. A new article of manufacture consisting of a sheet of paper impregnated with a mixture containing a vegetable oil and the polymerization products of the cumarone and indene groups. 10
9. A new article of manufacture consisting of a sheet of paper, having applied thereto a mixture containing China wood oil and the polymerization products of the cumarone and indene groups. 15
10. A new article of manufacture consisting of a sheet of paper, having applied thereto a mixture containing a vegetable oil and the polymerization products of the cumarone and indene groups. 20
11. A new article of manufacture consisting of a woven fabric, having applied thereto a mixture containing China wood oil and the polymerization products of the cumarone and indene groups, and having a coating of a similar mixture with or without a pigment therein. 25
12. A new article of manufacture consisting of a woven fabric, having applied thereto a mixture containing a vegetable oil and 30
- the polymerization products of the cumarone and indene groups, and having a coating of the polymerization products of the cumarone and indene groups, and having a coating of a similar mixture with or without a pigment therein. 35
13. A new article of manufacture consisting of a woven fabric of absorbent material, having applied thereto a mixture containing China wood oil and the polymerization products of the cumarone and indene groups, and having a coating of a similar mixture 40
- with or without a pigment therein. 45
14. A new article of manufacture consisting of a woven fabric of absorbent material, having applied thereto a mixture containing a vegetable oil and the polymerization products of the cumarone and indene groups, and having a coating of a similar mixture with or without a pigment therein. 50
15. A new article of manufacture consisting of a woven fabric coated with a mixture containing China wood oil and the polymerization products of the cumarone and indene groups. 55
16. A new article of manufacture consisting of a woven fabric coated with a mixture containing a vegetable oil and the polymerization products of the cumarone and indene groups.

In testimony whereof I affix my signature.  
ARMIN EICHLER.